

July 26, 1938.

W. J. MARSH

2,125,169

LUBRICANT OF HIGH FILM STRENGTH

Filed March 16, 1936



INVENTOR.

William J. Marsh  
BY

Kenneth E. Stewart  
ATTORNEY

## UNITED STATES PATENT OFFICE

2,125,169

## LUBRICANT OF HIGH FILM STRENGTH

William J. Marsh, Niagara Falls, N. Y., assignor to  
 Hooker Electrochemical Company, New York,  
 N. Y., a corporation of New York

Application March 16, 1936, Serial No. 69,011

10 Claims.

(Cl. 87—9)

It is now well known that the halogens, and more particularly chlorine, when introduced in very small quantities into lubricants, have the property of greatly increasing their film strength, i. e. the load carrying capacity of the lubricant. It is customary to introduce the chlorine by first combining it chemically with a suitable material, thus producing what is known as a "film-strengthening" agent. This agent is then added in minor proportion to the lubricating oil. For this purpose it is necessary to use a medium which is not itself incompatible with lubrication, and therefore hydrocarbons are now generally favored for this purpose. A great variety of hydrocarbons have been proposed, including members of the aliphatic, or paraffinic and olefinic group, the aromatic or carbon ring group, and the alicyclic or naphthenic group. These hydrocarbons are not, however, all equally suitable for the purpose. Some are difficult to chlorinate or incapable of accepting more than a small proportion of chlorine. Others when chlorinated are not sufficiently stable for the purposes intended. Still others are too stable, holding the chlorine so firmly that it cannot act effectively. Some are open to the further serious disadvantage that their chlorinated derivatives are of a very limited solubility in lubricating oils.

I have now discovered that certain new synthetic petroleum products, to be hereinafter described, which do not fall clearly within any of the above mentioned categories, possess unique properties as mediums for introduction of halogens into lubricating oil. For this purpose these products seem to combine most of the desirable characteristics of all the hitherto known hydrocarbons. I refer to the hydrogenation products of petroleum, now supplied commercially for use as solvents under the trade name "Solvesso". These petroleum hydrogenation products are made by subjecting light petroleum fractions to molecule-splitting conditions, such as pressures of the order of 3,000 lbs. or higher and temperatures of 300° C. or more, in the presence of hydrogen. A sulphur-resistant hydrogenation catalyst may also be employed. The process is so controlled that, notwithstanding the presence of hydrogen, the resulting product is hydrogen-unsaturated. The exact nature of the hydrogenation prod-

ucts referred to is not known, but it can be shown that neither the physical constants nor the chemical characteristics of these products correspond exactly to those of the aliphatic, aromatic or alicyclic series.

The physical characteristics of four typical examples of these petroleum hydrogenation products are as follows:

| Example No. | Sp. gr., 20/4° C. |       |        | Distillation range, degrees C. |       | 10 |
|-------------|-------------------|-------|--------|--------------------------------|-------|----|
|             | Initial           | Mean  | Final  | Initial                        | Final |    |
| 1.....      | 0.7567            | 0.784 | 0.8250 | 89                             | 145   | 15 |
| 2.....      | 0.8322            | 0.857 | 0.8744 | 136                            | 189   |    |
| 3.....      | 0.8733            | 0.897 | 0.9192 | 187                            | 218   |    |
| 4.....      | 0.9159            | 0.937 | 0.9500 | 214                            | 281   |    |

## Referring to the drawing:

This is a graphic comparison, upon the bases of specific gravities plotted against boiling points, of a large number of known hydrocarbons, with the petroleum hydrogenation products which I chlorinate and use in the lubricant of my invention.

At the extreme left of the sheet, curves 1 and 2 are plotted for the paraffines and olefines respectively. It will be seen that these form very definite, smooth curves, which tend to go to infinity, with a gravity of about 0.78 as an asymptote in both cases. Below these, curve 3 is similarly plotted for the naphthenes, cyclo-butane to cyclo-octane. It will be seen at a glance that this also is a definite, smooth curve, entirely distinct from the foregoing and having different characteristics in that, although it curves upward, it has no asymptote. Below this is curve 4, similarly drawn for cyclo-pentene and cyclo-hexene. Curve 5 is plotted for benzene, naphthalene and anthracene, which are aromatic hydrocarbons of one, two and three benzene rings respectively. This curve is very far from coinciding with any of the previous curves, but in common with them has an upward curving tendency. Curve 6 is plotted for benzene, toluene and xylene, which are substituted benzenes differing in that toluene has attached to it one methyl group and xylene two. This curve slopes in the reverse direction, i. e., boiling point decreases instead of increasing

5

20

25

30

35

40

45

50

with gravity as in the previous cases. Diphenyl, indene and retene form isolated points, having no near relatives.

Upon the same sheet the initial and final boiling points of the four typical petroleum hydrogenation products above referred to have been plotted against their corresponding specific gravities as indicated at 11, 12; 13, 14; 15, 16 and 17, 18 respectively. The two points so plotted for each product are joined by a dotted line. These dotted lines are designated as "product 1", "product 2", "product 3" and "product 4". Although these hydrogenation products are mixtures, the fractions for which the points are plotted, representing as they do the first and last 0.5 percent of each product respectively, have fairly sharp boiling points and therefore tend toward chemical individuals.

These points lie in a zone which is overlapped by the curve drawn for the naphthenes, cyclo-butane to cyclo-octane. However, this curve tends upward and its final portion points definitely away from this zone.

None of these points fall upon this or any other of the curves plotted for the known hydrocarbons. Therefore these terminal fractions are not identifiable as members of any well known groups of hydrocarbons; and since the terminal fractions are not readily classifiable, it is a fair presumption that some at least of the intermediate fractions are likewise unfamiliar compounds.

Moreover, these are not random mixtures. They are mixtures of hydrocarbons formed simultaneously under identical conditions and hence presumably closely related. They may be homologous. The resulting product therefore might be expected to show unique physical and chemical characteristics, and such is the case.

40 This is borne out by the following facts:

These petroleum hydrogenation products sulphonate freely. Since saturated hydrocarbons do not sulphonate this shows that to a large extent these products are more or less hydrogen-45 unsaturated. Moreover, this is also proven by the fact that they can be made to take up one to five percent of additional hydrogen. Since the paraffins and naphthenes are fully saturated compounds, the evidence of specific gravity and 50 boiling point that these products are not paraffins or naphthenes is thus definitely confirmed. These hydrogenation products chlorinate freely in light or darkness without the use of a catalyst and without foaming, whereas certain aliphatic 55 hydrocarbons, such as petrolatum, foam so badly during chlorination that the operation becomes one of great difficulty. Although non-volatile, they readily take up chlorine to a chlorine content of 60 percent or more by weight, without 60 the use of a solvent to keep them in fluid condition during the process. In this respect they resemble the paraffins more than the carbon-ring compounds, which, unless they are chlorinated with a catalyst, produce unstable addition 65 compounds. These products differ from the paraffins, however, in that paraffins, the chains of which are long enough to be non-volatile, become so viscous when they have taken up chlorine to a content of 40 to 45 percent by weight

70 that, unless they are dissolved in a solvent, the chlorination cannot be further continued. During chlorination of these products HCl is given off copiously, showing that the reaction is largely a substitution. When freed from this HCl they 75 remain substantially neutral during prolonged

storage at ordinary temperatures, even under actinic light, whereas chlorinated aliphatic hydrocarbons, although stable in darkness, tend to give off HCl when exposed to light.

These petroleum hydrogenation products when chlorinated are yellowish brown, viscous, oily liquids, of a lighter color, however, than the chlorinated paraffins containing a comparable percentage of chlorine. They have no definite solidifying point, but upon cooling become more and more viscous until finally they practically cease to flow; but they do not become true solids at temperatures attainable by ordinary means. They do not become waxy and never contain more crystals than could be accounted for by 15 traces of impurities. In these respects again they resemble the chlorinated paraffins and are in sharp contrast with the chlorinated carbon-ring compounds. These latter, in general, are characterized by sharp melting points. At ordinary temperatures they are generally either non-viscous, non-oily liquids or waxy crystalline solids. This is especially true of the chlorinated benzenes and substituted benzenes. When chilled, with or without seeding, they can always be 25 made to yield crystals, with liberation of the latent heat of the liquid. The diphenyls, in some grades, are viscous, but they are sticky or syrupy rather than oily, and tend to cause a notable increase in friction.

These chlorinated petroleum hydrogenation products containing 60 percent chlorine or over are miscible at room temperature and higher in all proportions with lubricating oils. In this respect again they are like the chlorinated paraffinic hydrocarbons containing 30 to 45 percent chlorine and in sharp contrast with the chlorinated carbon-ring carbons, some of which are of very limited solubility in oils. Thus tetrachlor and hexachlor benzene, containing respectively 40 65.7 and 74.6 percent of chlorine, have a limit of solubility in oils of only about 2 percent. Chlor-naphthalene and chlor-diphenyl, containing 56 and 68 percent of chlorine, have limits of solubility in oils of 9 and 7 percent respectively. Hexa-45 chlor-ethane, which contains 90 percent chorine, has a solubility in oils of about 9 percent.

These hydrogenation products may be chlorinated at temperatures up to 190° C., as compared with a limit of 130° C. in the case of paraffins. 50 This, of course, means that they are stable at a correspondingly higher temperature.

The fact that the chlorination of these hydrogenation products, as stated above, is largely a substitution precludes the theory that they are 55 simple olefines. Moreover, chlorinated olefines have physical characteristics similar to those of paraffins of the same number of carbon atoms and chlorine content. That is to say, olefines have substantially the same limits of chlorine 60 content as the corresponding paraffins and the same gravity and decomposition temperature when chlorinated, in both of which respects they are quite different from any chlorinated carbon-ring compounds.

To recapitulate, these petroleum hydrogenation products differ from the paraffins in that

(a) They are largely unsaturated compounds, whereas paraffins are fully saturated.

(b) Their gravities for given boiling points are 70 much higher.

(c) They readily take up chlorine to a chlorine content of 60 percent or more by weight without becoming so viscous as to require the use of a solvent, whereas the non-volatile paraffins take 75

up chlorine to a content of not more than 45 percent under similar circumstances.

(d) These petroleum hydrogenation products may be chlorinated at 190° C. as compared with 5 a limit of 130° C. for the paraffins.

These hydrogenation products differ from the olefines in that

(a) They chlorinate largely by substitution. 10 (b) Their gravities are much higher for a given boiling point.

(c) They take up more chlorine than chlorinated olefines, as indicated under the above comparison for paraffins.

These hydrogenation products differentiate 15 from naphthenes in that

(a) They are largely unsaturated compounds, whereas naphthenes are fully saturated.

(b) They have a higher range of both gravity and boiling point.

20 These hydrogenation products differ from all well known carbon-ring compounds in that

(a) Their gravities and boiling points do not correspond to those of any known ring compounds.

25 (b) They chlorinate freely in the light or dark, without a catalyst, and without producing the unstable addition compounds obtained if known carbon-ring compounds are chlorinated under similar conditions.

30 (c) The chlorinated hydrogenation products are miscible with lubricating oils at room temperature in all proportions, whereas the chlorinated carbon-ring compounds have upper limits of solubility in such oils of from 2 to 9 percent.

35 (d) The chlorinated hydrogenation products are viscous, oily liquids at ordinary temperatures, having no definite solidifying point, and never becoming true solids, whereas the chlorinated carbon-ring compounds pass sharply from non-oily liquids to waxy, crystalline solids, with lib- 40 eration of the latent heat of the liquid.

In short, these hydrogen-unsaturated petroleum hydrogenation products are probably hitherto unknown members or mixtures of the 45 almost infinitely diversified family of hydrocarbons.

These petroleum hydrogenation products, especially those in the lower boiling ranges, when chlorinated to less than 50 percent chlorine, 50 have an extremely unpleasant odor and irritant effect upon the skin. This may be due to sulphur and nitrogen derivatives. I have discovered, however, that when the chlorination is carried beyond 50 percent this odor is destroyed and the irritant effect ceases.

55 These petroleum hydrogenation products therefore combine the most desirable properties of the aliphatic, alicyclic and carbon-ring hydrocarbons heretofore known, namely ease of chlorination to a high chlorine content, resulting in a sparklingly clear product, of light color and unlimited solubility in oils which will not cause turbidity in the oil and of good stability under heat. Moreover, when used in lubricants they have exceptional merit as film-strengthening agents. This 60 is shown by the following tests:

#### Example

Many tests of Pennsylvania Bright Stock lubricating oil upon the Floyd lubricant testing machine show that this oil fails at an average load of about 140 lbs. upon the gauge of this machine. To this oil was added in various proportions chlorinated "Solvesso" boiling before 70 chlorination between 136° C. and 189° C., and

containing various percentages of chlorine. The test results were as follows:

| Proportion of chlorinated product, percent | Chlorine content of chlorinated product, percent | Test results                                     | 5  |
|--------------------------------------------|--------------------------------------------------|--------------------------------------------------|----|
| 6                                          | 30                                               | Failed at 600 lbs. gauge in 40 seconds.          |    |
| 3                                          | 50                                               | Withstood 600 lbs. for 1 minute without failure. | 10 |
| 4                                          | 50                                               | Do.                                              |    |
| 5                                          | 50                                               | Do.                                              |    |
| 2                                          | 60                                               | Do.                                              |    |
| 3                                          | 60                                               | Do.                                              |    |

These comparative tests show that the addition 15 of 1.5 to 1.8 percent of chlorine in combination with these petroleum hydrogenation products increased the film strength of the base oil from 140 lbs. upon the gauge so that it was able to withstand the full limit of the machine of 600 20 lbs. upon the gauge without failure. These results are distinctly superior to those obtainable with the well known film strengthening agents, such as chlorinated paraffins, chlorinated naphthalene, etc., none of which consistently carry a 25 load of much over 400 lbs. upon the gauge of the Floyd testing machine under the conditions of the above tests.

Upon the drawing the initial and final boiling 30 points of the first and fourth products have been plotted against their means specific gravities, as indicated at 7, 8, 9 and 10. The initial boiling points and final boiling points of the two products respectively have been joined by dotted lines, which, with the two limiting gravities, form a 35 quadrilateral enclosing an area within which the four products are largely comprised. This area graphically defines by their gravities and boiling points substantially all the petroleum hydrogenation products coming within the scope 40 of my invention.

Point 7 of this quadrilateral appears to fall upon curve 3, but this has no significance as point 7 is not drawn for a chemical individual. Furthermore, it represents an unsaturated compound which could not be a naphthene. Points 45 11 and 18 fall outside the quadrilateral. This again has no significance as their points represent the fractions that are very nearly chemical individuals. Thus, point 18 represents the boiling 50 point of the final fraction of product No. 4, plotted against its actual specific gravity, whereas point 9 represents the boiling point of the same fraction plotted against the mean gravity of the product as a whole.

In the following claims the expression "relatively stable" means more heat stable than the hitherto known oil-miscible addition agents for lubricants.

60 I claim as my invention:

1. A lubricant composition of relatively high film strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such as would be produced by chlorinating a hydrogen - unsaturated petroleum hydrogenation 70 product having a gravity above 0.78 and boiling between 89° C. and 281° C., such as would be produced by subjecting a light petroleum fraction to molecule-splitting conditions of temperature and pressure in presence of hydrogen. 75

2. A lubricant composition of relatively high film-strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such as would be produced by chlorinating a 5 sulphonatable hydrocarbon having a gravity above 0.78 and boiling between 89° C. and 281° C., such as would be produced by subjecting a light petroleum fraction to molecule-splitting conditions of temperature and pressure in presence of 10 hydrogen.
- 15 3. A lubricant composition of relatively high film strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such as would be produced by chlorinating a 20 hydrocarbon capable of taking up 1 to 5 per cent of its weight of hydrogen having a gravity above 0.78 and boiling between 89° C. and 281° C., such as would be produced by subjecting a light petroleum fraction to molecule-splitting conditions 25 of temperature and pressure in presence of hydrogen.
- 25 4. A lubricant composition of relatively high film strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such 30 as would be produced by chlorinating a hydro- 35 gen-unsaturated petroleum hydrogenation product having a gravity of substantially 0.855 and boiling between 136° C. and 189° C., such as would be produced by subjecting a light petroleum 40 fraction to molecule-splitting conditions of temperature and pressure in presence of hydrogen.
- 45 5. A lubricant composition of relatively high film strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such 50 as would be produced by chlorinating a hydro- 55 gen-unsaturated petroleum hydrogenation product having a gravity of substantially 0.987 and boiling between 187° C. and 218° C., such as would be produced by subjecting a light petroleum 55 fraction to molecule-splitting conditions of temperature and pressure in presence of hydrogen.
- 55 6. A lubricant composition of relatively high film strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such 60 as would be produced by chlorinating a hydro- 65 gen-unsaturated petroleum hydrogenation product having a gravity of substantially 0.937 and boiling between 214° C. and 281° C., such as 70

would be produced by subjecting a light petroleum fraction to molecule-splitting conditions of temperature and pressure in presence of hydrogen.

7. A lubricant composition of relatively high film strength comprising a major proportion of a mineral lubricating oil and a minor proportion of an oily, liquid, relatively stable, substantially neutral and non-volatile chlorination product, miscible in all proportions at ordinary temperatures with said oil and containing not less than 45 per cent of largely substituted chlorine, such as would be produced by chlorinating a hydro- 10 gen-unsaturated petroleum hydrogenation product having a boiling range which when plotted 15 against the gravity of said product falls within the quadrilateral formed by lines joining the four points plotted respectively for a gravity of 0.784 against boiling points of 89° C. and 145° C. and a gravity of 0.937 against boiling points 20 of 214° C. and 281° C., such as would be produced by subjecting a light petroleum fraction to molecule-splitting conditions of temperature and pressure in presence of hydrogen.

8. A lubricant composition of relatively high film strength comprising a major proportion of a mineral lubricating oil and a minor proportion of an oily, liquid, relatively stable, non-irritating, substantially neutral and non-volatile chlorination product, miscible in all proportions at 30 ordinary temperatures with said oil, such as would be produced by chlorinating to not less than 50 per cent of largely substituted chlorine a hydro-unsaturated petroleum hydrogenation product having a gravity above 0.78 and 35 boiling between 89° C. and 281° C., such as would be produced by subjecting a light petroleum fraction to molecule-splitting conditions of 40 temperature and pressure in presence of hydrogen.

9. A lubricant composition of relatively high film-strength comprising a major proportion of a mineral lubricating oil and a minor proportion of an oily, liquid, relatively stable, substantially neutral and non-volatile chlorination product, miscible in all proportions at ordinary temperatures with said oil, such as would be produced by chlorinating at a temperature of 130° C. to 190° C., regardless of light and in the absence of any catalyst a hydro-unsaturated 45 petroleum hydrogenation product, such as would be produced by subjecting a light petroleum fraction to molecule-splitting conditions of 50 temperature and pressure in presence of hydrogen.

10. The process for production of a lubricant 55 composition of relatively high film strength comprising passing chlorine into a hydro-unsaturated petroleum hydrogenation product having a gravity above 0.78 and boiling between 89° C. and 281° C., such as would be produced by sub- 60 jecting a light petroleum fraction to molecule- splitting conditions of temperature and pressure in presence of hydrogen, at a temperature between 130° C. and 190° C., regardless of light and in the absence of any catalyst and removing 65 the hydrogen chloride formed by the reaction, whereby there results an oily, liquid, relatively stable, substantially neutral and non-volatile chlorination product, miscible in all proportions at ordinary temperatures with mineral lubricat- 70 ing oil, and adding a minor proportion of said chlorination product to a major proportion of said mineral lubricating oil.